

Patented Jan. 14, 1936

2,028,000

# UNITED STATES PATENT OFFICE

2,028,000

## PERMANENT MAGNET CONTAINING NICKEL, ALUMINUM, AND VANADIUM

Tokushichi Mishima, Yodobashi-ku,  
Tokyo, Japan

No Drawing. Original application January 20, 1932, Serial No. 587,822. Divided and this application August 7, 1935, Serial No. 35,209. In Japan August 27, 1931

### 4 Claims. (Cl. 175—21)

This invention relates to a strong permanent magnet and forms a divisional from the copending application Serial No. 587,822 filed January 20, 1932.

This permanent magnet contains the main elements iron, nickel and aluminum with iron as the basic element, 5 to 40% nickel, 7 to 20% aluminum; and the auxiliary element vanadium from trace to 10% with or without carbon from trace to 1.5%.

10 In original application 587,822 it is described that a so-called "irreversible nickel steel" can be changed into a "reversible steel" by the addition of aluminum, thereby obtaining a strong magnetic alloy. According to the invention it has been found that the addition of a proper amount of other metals as auxiliary elements will further improve the magnetic properties as well as the tenacity and ductility of the permanent magnet and facilitate the mechanical working of the magnet.

15 It is well known that the more minute the micro-structure of the magnet steels is, the greater is the increase in the number of molecular magnets arranged irregularly at the boundaries of the crystal grains so that consequently the coercive force and the residual magnetism also increase. This feature is gained by the addition of certain amounts of one or more auxiliary metals to the main elements iron, nickel and aluminum in the proportions herein given.

20 According to this invention it has been found that the new alloy as mentioned above, can further be improved by the addition of vanadium of below 10%. By this means, the magnetic prop-

erties become still further increased and the forging and rolling properties are considerably improved.

Actual examples for this case are given below:

| Chemical composition (%) |        |          |          | Magnetic properties         |                                 |
|--------------------------|--------|----------|----------|-----------------------------|---------------------------------|
| Iron                     | Nickel | Aluminum | Vanadium | Coercive force (Hc) (gauss) | Residual magnetism (Br) (gauss) |
| 65.5                     | 24.0   | 10.0     | 0.4      | 280                         | 9,700                           |
| 58.5                     | 30.0   | 12.0     | 1.5      | 480                         | 9,500                           |
| 63.0                     | 23.0   | 9.5      | 4.5      | 290                         | 9,400                           |

It is also noted in this case that the presence of carbon of below 1.5% and/or a small amount of impurities does not materially affect the magnetic properties of the alloy.

I claim:

1. A permanent magnet comprising 5 to 40% nickel, 7 to 20% aluminum, from trace to 10% vanadium, and the remainder iron.

2. A permanent magnet comprising 5 to 40% nickel, 7 to 20% aluminum, from trace to 10% vanadium, and the remainder substantially iron.

3. A permanent magnet comprising 5 to 40% nickel, 7 to 20% aluminum, from trace to 10% vanadium, from trace to 1.5% carbon and the remainder iron.

4. A permanent magnet comprising 5 to 40% nickel, 7 to 20% aluminum, from trace to 10% vanadium, from trace to 1.5% carbon and the remainder substantially iron.

TOKUSHICHI MISHIMA.